# EUROPEAN PATENT APPLICATION

(11) **EP 0 371 927 A1**
(43) Date of publication of application: **06.06.1990**
(21) Application number: 89830489.4
(22) Date of filing: 10.11.1989
(51) Int. Cl.: C25B 1/00

(54) **A method of obtaining stannous sulphate, and equipment for the implementation of such a method**

(30) Priority: 16.11.1988 IT 4016788
(71) Applicant: Garuti, Giuseppe, I-41100 Modena (IT)
(72) Inventor: Garuti, Giuseppe, I-41100 Modena (IT)
(74) Representative: Lanzoni, Luciano

(57) **Abstract**

The process is electrolytic, making use of a tin anode (5), and a cathode (4) of conductive material resistant to sulphuric acid, which are immersed in a bath of dilute sulphuric acid separated into anode and cathode regions by a diaphragm (6) that allows the passage of negatively-charged ions only; the equipment consists in an electrolytic cell (1) with lead, titanium or graphite cathodes (4) and generously proportioned flat tin anodes (5), in which cathode and anode compartments (2, 3) are created by the addition of a separation barrier fabricated with at least part of its structure providing the diaphragm (6).

## Description

The present invention relates to a method of obtaining stannous sulphate, and to equipment for the implementation of such a method.

Among its various uses, stannous sulphate serves as a colouring agent for aluminium, which acquires a particular bronze-like aspect when treated with the chemical.

Conventionally, stannous sulphate is obtained by means of a procedure that involves the reaction of powdered tin with hydrochloric acid; this gives stannous chloride, to which sulphuric acid is then added so as to bring about the precipitation of stannous sulphate, the sulphate being less soluble than the chloride.

The precipitate obtained by such a method contains impurities in the form of chlorides which adversely affect the colouring treatment referred to above, and must therefore be removed completely.

The cost of stannous sulphate mnufactured in this conventional manner is high enough, especially when compared with that of the raw tin, but rises still further when supplied to end users in solution, for reasons of convenience.

The object of the present invention is to overcome the drawbacks thus described through the provision of a method, and of equipment for its application, by means of which to obtain stannous sulphate that is free from unwanted impurities (chlorides), and less costly than the product given by conventional methods currently in use, as referred to above. The stated object, and other objects besides, can be realized with a method as characterized in the appended claims. Such a method consists essentially in a process of electrolysis involving the use of an anode fashioned from tin, and a cathode embodied in a conductive material unaffected by sulphuric acid; these are immersed in a solution of sulphuric acid, and the anode and cathode regions separated by a diaphragm permeable to negative ions only. In like manner, the same objects are realized with equipment as characterized in the claims appended, which consists in an electrolytic cell comprising at least one cathode embodied in material that will conduct electricity while remaining unaffected by sulphuric acid, at least one anode embodied in tin, and a barrier, separating the compartments occupied by the anode and cathode, of which at least a part is embodied as a diaphragm permeable exclusively to negative ions.

The invention will now be described in detail, by way of example, with the aid of the accompanying sheet of drawings, in which:
-fig 1 is a schematic illustration of equipment according to the invention, viewed from above;
-fig 2 is the section through II-II in fig 1.

The method disclosed consists essentially in a process of electrolysis, implemented as described in the following specification. Whilst reference is made throughout the description to a non-continuous type of process, such modifications as would serve to render the cycle continuous remain comfortably within the capabilities of a person skilled in the art.

An electrolytic cell is prepared, with a tin anode, and a cathode embodied in a material such as lead, titanium or graphite, or indeed any given material that will conduct electricity and at the same time remain unaffected by exposure to sulphuric acid; the electrolyte in which the anode and cathode are immersed is in fact a solution of sulphuric acid.

The anode and the cathode region are separated as compartments by means of a diaphragm, conventional in embodiment, which can be permeated by negatively charged ions only and thus disallows the passage of positive ions.

Initial concentrations of sulphuric acid in the two electrode compartments of the cell are dissimilar -viz, 100...200 g/l in the cathode compartment and 50...100 g/l in the anode.

In addition, the anode region is supplemented with tartaric acid in a concentration of 1...10 g/l, in order to prevent the precipitation of any stannic oxide (SnO₂, the tetravalent tin oxide) that may be formed; at all events, the concentration must be kept below 10 g/l, since excess tartaric acid will give rise to the formation of stannous tartrate, ultimately producing a material that is unsuitable for use and can only be jettisoned.

Electrolysis is induced with a power supply input of between 1.5 and 4 V d.c. (approx), with current of between 250 and 350 A per m² of diaphragm area; the voltage should be no higher however, as values in excess of 4 V can give place to the formation of stannic oxide as well as causing mechanical damage to the diaphragm.

With voltages higher than 2 V, provision should be made for cooling the electrolyte, especially in the cathode compartment; during electrolysis, in fact, heat is generated that could raise the temperature of the solution and damage the diaphragm.

Preferably, the electrolyte will be maintained at a temperature below 40 °C.

Equipment suitable for implementation of the method disclosed comprises an electrolytic cell 1 provided with two centrally positioned cathodes 4 embodied in lead, or titanium or graphite, and two anodes 5 embodied in tin, located externally of the cathodes one on either side. In order to increase the anodic surface area bathed by the electrolyte, and thus enhance the take-up of positively-charged bivalent tin ions in the solution, the relative electrodes 5 will be of flat embodiment (tin sheet or ingots), or fashioned from scrap tin.

The cell comprises means by which to separate the cathode compartment 2 from the anode compartment 3, which completely encompass the cathode compartment and consist in two diaphragms 6 carried between two supports 7; more exactly, the two diaphragms 6 are located each between one cathode 4 and the relative anode 5 and are permeable to negative ions only. 8 denotes a cooling system located in the cathode compartment 2, illustrated schematically as a coil, fashioned in lead, into which a flow of liquid coolant is directed. A similar system might also be installed in the anode compartment 3.

The process according to the method disclosed is implemented as follows.

With the d.c. voltage applied to the cell, positive bivalent tin ions are taken up by the electrolyte in the anode compartment, and hydrogen is produced in the cathode compartment. Positive Sn ions taken into solution during electrolysis are retained in the anode compartment by the diaphragms 6 (being impenetrable to positively-charged ions), and thus prevented from crossing to the cathode compartment; the barrier thus created is in fact essential to the successful outcome of the process, as without the diaphragm 6, positive Sn ions would migrate toward the cathode 4, depositing on and smothering its surface in a short time.

SO₄-- ions, on the other hand, are able to migrate freely from the cathode compartment to the anode. Accordingly, as the process continues, one has formation in the anode compartment of a solution rich both in positive Sn ions and in SO₄-- ions.

The process is stopped when the concentration of stannous sulphate in the electrolyte occupying the anode compartment 3 registers at 150...200 g/l. This is a preferred juncture at which to call a halt, as higher concentrations will both lower the conductivity of the electrolyte, thus reducing the efficiency of the process, and create conditions in which oxidation of the tin in solution can occur. The solution taken from the electrolytic cell, at the juncture in question, is ready for immediate sale.

Whilst the final solution may well contain excess sulphuric acid, especially where the concentration of the acid is maintained high initially in the cathode compartment, this constitutes no drawback whatever as regards use of the stannous sulphate solution as a colouring agent for aluminium.

## Claims

1) A method of obtaining stannous sulphate,
characterized
in that it involves a process of electrolysis utilizing a tin anode, and a cathode embodied in material capable both of conducting electricity and of remaining unaffected by exposure to sulphuric acid, which are immersed in a solution of sulphuric acid separated into respective anode and cathode regions by a diaphragm of conventional embodiment that is permeable to negatively-charged ions only.

2) A process as in claim 1, wherein electrolysis is induced by applying a direct voltage of 1,5...4 V and initial current of 250...350 A per m² of the diaphragm surface area.

3) A process as in claim 1, wherein the electrolyte contains initial sulphuric acid concentrations of 50...100 g/l in the anode region and 100...200 g/l in the cathode region.

4) A process as in claim 1, wherein tartaric acid is added to the electrolyte occupying the anode region in a concentration of between 1 and 10 g/l.

5) A process as in claim 1, comprising the step of cooling the electrolyte.

6) Equipment for obtaining stannous sulphate by way of the process of claim 1,
characterized
in that it consists in an electrolytic cell (1) which comprises at least one cathode (4) embodied in a conductive material unaffected by sulphuric acid and at least one anode (5) fashioned from tin, and is separated into distinct cathode and anode compartments (2, 3) by means embodied at least in part as a conventional diaphragm (6) permeable to negatively-charged ions only.

7) Equipment as in claim 6, wherein the electrolytic cell comprises two centrally located cathodes (4), and two anodes (5) located externally of the two cathodes on either side, such that the separation means encompass the cathodes and are arranged with their diaphragm area directed toward the anodes.

8) Equipment as in claim 6, comprising a cooling system (8) immersed in the electrolyte.
